



US010731259B2

(12) **United States Patent**  
**Koeberlein et al.**

(10) **Patent No.:** **US 10,731,259 B2**  
(45) **Date of Patent:** **Aug. 4, 2020**

(54) **PISTONS WITH THERMAL BARRIER COATINGS**

(71) Applicant: **CUMMINS INC.**, Columbus, IN (US)

(72) Inventors: **David E. Koeberlein**, Columbus, IN (US); **J. Steven Kolhouse**, Columbus, IN (US); **Michael Hays**, Columbus, IN (US)

(73) Assignee: **Cummins Inc.**, Columbus, IN (US)

(\*) Notice: Subject to any disclaimer, the term of this patent is extended or adjusted under 35 U.S.C. 154(b) by 52 days.

(21) Appl. No.: **15/898,047**

(22) Filed: **Feb. 15, 2018**

(65) **Prior Publication Data**

US 2018/0179644 A1 Jun. 28, 2018

**Related U.S. Application Data**

(63) Continuation-in-part of application No. 15/796,302, filed on Oct. 27, 2017.

(Continued)

(51) **Int. Cl.**

**F02B 75/28** (2006.01)  
**F02F 3/12** (2006.01)

(Continued)

(52) **U.S. Cl.**

CPC ..... **C23C 28/042** (2013.01); **C23C 4/01** (2016.01); **C23C 4/02** (2013.01); **C23C 4/11** (2016.01);

(Continued)

(58) **Field of Classification Search**

CPC ..... F02F 3/12; F02F 3/22; F05C 2251/048;

F02M 61/14; F02B 77/11; F02B 75/28; C23C 28/042; C23C 4/01; C23C 4/02; C23C 4/11; C23C 4/134; C23C 4/129; F01B 7/14

See application file for complete search history.

(56)

**References Cited**

**U.S. PATENT DOCUMENTS**

5,560,283 A 10/1996 Hannig  
6,256,984 B1 7/2001 Voss et al.  
(Continued)

**FOREIGN PATENT DOCUMENTS**

CN 102226427 10/2011

**OTHER PUBLICATIONS**

Non-Final Office Action on U.S. Appl. No. 15/796,302 dated Aug. 28, 2019.

(Continued)

*Primary Examiner* — David P Bryant

*Assistant Examiner* — Lee A Holly

(74) *Attorney, Agent, or Firm* — Foley & Lardner LLP

(57) **ABSTRACT**

A method of making a piston for an opposed-piston engine comprises providing a piston. The piston comprises a substantially cylindrical portion including a sidewall and a piston crown located at an end of the piston. The piston crown comprises an end surface structured to form a combustion chamber when disposed within a cylinder bore in cooperation with an end surface of a cooperating opposing piston. A bonding layer including a bonding material is deposited on the end surface of the piston crown using a high velocity oxy-fuel spray process. At least one thermal barrier layer comprising ceramic material is deposited above the bonding layer.

**11 Claims, 11 Drawing Sheets**



**Related U.S. Application Data**

|      |                                                                |  |                  |                  |                                      |
|------|----------------------------------------------------------------|--|------------------|------------------|--------------------------------------|
| (60) | Provisional application No. 62/417,463, filed on Nov. 4, 2016. |  | 9,163,505 B2     | 10/2015          | Dion                                 |
|      |                                                                |  | 9,810,174 B2     | 11/2017          | Wahl                                 |
|      |                                                                |  | 2006/0042575 A1  | 3/2006           | Schmuecker et al.                    |
|      |                                                                |  | 2007/0084449 A1  | 4/2007           | Najt et al.                          |
|      |                                                                |  | 2010/0326394 A1  | 12/2010          | Hofbauer                             |
|      |                                                                |  | 2011/0114038 A1  | 5/2011           | Lemke                                |
|      |                                                                |  | 2011/0271932 A1  | 11/2011          | Fuqua                                |
|      |                                                                |  | 2012/0080004 A1  | 4/2012           | Menezes                              |
|      |                                                                |  | 2013/0112175 A1  | 5/2013           | Wahl et al.                          |
|      |                                                                |  | 2013/0220115 A1  | 8/2013           | Kantola                              |
|      |                                                                |  | 2014/0090625 A1  | 4/2014           | Dion et al.                          |
|      |                                                                |  | 2014/0102294 A1  | 4/2014           | Klein                                |
|      |                                                                |  | 2014/0196439 A1  | 7/2014           | Dolan et al.                         |
|      |                                                                |  | 2014/0255617 A1  | 9/2014           | Sasaki                               |
|      |                                                                |  | 2015/0252715 A1  | 9/2015           | MacKenzie                            |
|      |                                                                |  | 2016/0069293 A1  | 3/2016           | McClearen et al.                     |
|      |                                                                |  | 2016/0252065 A1* | 9/2016           | Johnson ..... F02M 61/14<br>123/51 R |
|      |                                                                |  |                  | 2017/0145914 A1* | 5/2017 Lineton ..... F02B 77/11      |
|      |                                                                |  |                  | 2017/0254261 A1  | 9/2017 Morton et al.                 |
|      |                                                                |  |                  | 2017/0335752 A1  | 11/2017 Morton                       |

**(56) References Cited**

## U.S. PATENT DOCUMENTS

7,549,401 B2 6/2009 Lemke  
8,087,389 B2 1/2012 Lemke

## OTHER PUBLICATIONS

Non-Final Office Action on U.S. Appl. No. 15/809,358 dated Jul. 30, 2018.

\* cited by examiner



四



FIG. 2



FIG. 3A



FIG. 3C



三三  
三  
三



FIG. 4



FIG. 5

FIG. 6



**FIG. 7**

**FIG. 8**

**FIG. 9**

FIG. 10



## PISTONS WITH THERMAL BARRIER COATINGS

### CROSS-REFERENCE TO RELATED APPLICATIONS

This application is a Continuation-in-part application of U.S. patent application Ser. No. 15/796,302, filed Oct. 27, 2017 and entitled, "PISTONS WITH THERMAL BARRIER COATINGS FOR OPPOSED-PISTON ENGINES," which claims the benefit of priority to U.S. Provisional Patent Application No. 62/417,463, filed on Nov. 4, 2016, titled "PISTONS WITH THERMAL BARRIER COATINGS FOR OPPOSED-PISTON ENGINES," the entire disclosures of which are hereby incorporated by reference in their entirety.

### RELATED APPLICATIONS

This Application contains subject matter related to the subject matter of U.S. Provisional Application No. 62/417,499, filed Oct. 27, 2017 and titled "PISTONS WITH THERMAL BARRIER COATINGS FOR OPPOSED-PISTON ENGINES," and U.S. patent application Ser. No. 15/809,358, filed Nov. 10, 2017, and titled "PISTONS WITH THERMAL BARRIER COATINGS FOR OPPOSED-PISTON ENGINES," which is a continuing application of U.S. patent application Ser. No. 15/796,302, the disclosures of which are incorporated herein by reference in their entirety.

### STATEMENT REGARDING FEDERALLY SPONSORED RESEARCH

This invention was made with government support under NAMC Project Agreement No. 69-201502 awarded by the NATIONAL ADVANCED MOBILITY CONSORTIUM (NAMC), INC. The government has certain rights in the invention.

### FIELD

The present disclosure relates to piston thermal management constructions for uniflow-scavenged opposed-piston, internal combustion engines.

### BACKGROUND

When compared to conventional "Vee" and straight-inline internal combustion engines with a single piston in each cylinder, opposed-piston engines possess architectural advantages in thermodynamics and combustion that can deliver improvements in measures of engine performance. However, uniflow-scavenged, opposed-piston engines characteristically have thermal requirements that are different from engines that have one piston per cylinder, and thus thermal management techniques differ. The difference in thermal requirements occurs in uniflow-scavenged opposed-piston engines due to the nature of charge air flow into and exhaust flow from the cylinders in these engines.

During scavenging in a uniflow-scavenged, opposed-piston engine, the predominant fluid flow is unidirectional, that is to say, charge air flows through the intake port of a cylinder and exhaust flows out of the cylinder's exhaust port. Because the air entering the cylinder is cooler than the exhaust, the exhaust portion of the cylinder and the exhaust piston that moves across the exhaust port are exposed to greater heat and higher temperatures than the intake portion

of the cylinder and the intake piston that moves across the intake port. Thus, the unidirectional flow of air and exhaust leads to exposure of the opposite ends of a cylinder to different temperature profiles. Additionally, in a two-stroke cycle of uniflow-scavenged, opposed-piston engines, there is less time for piston cooling between firing or combustion events, so the difference in thermal environments that the exhaust and intake pistons are exposed to is even more pronounced as compared to engines that have one piston per cylinder.

### SUMMARY

In some embodiments of the present disclosure, a piston for use in an opposed-piston internal combustion engine comprises a substantially cylindrical portion including a sidewall. The piston further comprises a piston crown located at an end of the piston, the piston crown comprising an end surface structured to form a combustion chamber when disposed within a cylinder bore in cooperation with an end surface of a cooperating opposing piston, the piston crown further comprising titanium or a titanium alloy. The piston also comprises a thermal barrier coating on the piston crown.

In a set of embodiments, a method of making a piston for an opposed-piston engine comprises providing a piston. The piston comprises a substantially cylindrical portion including a sidewall and a piston crown located at an end of the piston. The piston crown comprises an end surface structured to form a combustion chamber when disposed within a cylinder bore in cooperation with an end surface of a cooperating opposing piston. A bonding layer including a bonding material is deposited on the end surface of the piston crown using a high velocity oxy-fuel spray process. At least one thermal barrier layer comprising ceramic material is deposited above the bonding layer.

In another set of embodiments, a method of making a piston for an opposed-piston engine comprises providing a piston. The piston comprises a substantially cylindrical portion including a sidewall and a piston crown located at an end of the piston. The piston crown comprises an end surface structured to form a combustion chamber when disposed within a cylinder bore in cooperation with an end surface of a cooperating opposing piston. A portion of the end surface is masked. A bonding layer including a bonding material is deposited on the end surface of the piston crown. The portion of the end surface is unmasked. Furthermore, the bonding layer is deposited on at least the portion of the end surface for a first predetermined time. At least one thermal barrier layer comprising ceramic material is deposited above the bonding layer.

The following features may be combined in any suitable manner in the piston, the uniflow-scavenged opposed-piston engine, and/or the method described herein. The features for adapting to variations in thermal conditions between the intake and exhaust end may include the use of different materials for an exhaust piston from those used for an intake piston in the uniflow-scavenged opposed-piston engine. The materials used for the exhaust piston may include materials that have high strength at high temperature, materials that have a small coefficient of thermal expansion, and/or materials that are poor conductors of heat. In some implementations, the crown of the exhaust piston may be made of a different material than the crown of the intake piston; for example the material may include a material that has high strength at high temperature, a material that has a small coefficient of thermal expansion, and/or a material that is a

poor conductor of heat (e.g., a thermal insulator). The material used for portions of or all of the exhaust piston, such as for the exhaust piston's crown, that is different from the material used for the intake piston, can include in some embodiments titanium, a titanium alloy, nickel, a nickel alloy, a ceramic material, a composite material (e.g., a glass or ceramic reinforced polymer composite), a cermet, or a combination of two or more of these. The exhaust piston can have a thermal barrier coating, and in some implementations, the thermal barrier coating can be a layer of a single material or the thermal barrier coating can include multiple layers of two or more materials. In some embodiments, the exhaust piston comprises a titanium alloy with a ceramic coating that comprises yttria stabilized zirconia.

#### BRIEF DESCRIPTION OF THE DRAWINGS

FIG. 1 depicts a side elevation view of an example arrangement of cylinders, pistons, and a gear train in an opposed-piston engine.

FIG. 2 depicts a longitudinal cross-sectional view of an example of a cylinder of an opposed-piston engine constructed for two stroke-cycle operation.

FIG. 3A depicts an example exhaust piston for a uniflow-scavenged opposed-piston engine.

FIGS. 3B and 3C depict cross-sectional representations of the example exhaust piston shown in FIG. 3A.

FIG. 4 depicts a cross-sectional view of a portion of an example exhaust piston with an example thermal barrier coating.

FIG. 5 shows a flow chart for an example method for forming a thermal barrier coating on an exhaust piston for use with an opposed-piston engine.

FIG. 6 is a flow chart of another example method for forming a thermal barrier coating on an exhaust piston for use with an opposed-piston engine.

FIG. 7 is a perspective image of an example exhaust piston for a uni-flow scavenged opposed-piston engine, according to another embodiment.

FIG. 8 is an image of an assembly for depositing a bonding layer and/or a thermal barrier layer on an end surface of a piston, according to a particular embodiment.

FIG. 9 is a top view of an end surface of the piston of FIG. 7 with a portion of the end surface covered by a mask.

FIG. 10 is a flow chart of yet another example method for forming a thermal barrier coating on an exhaust piston for use with an opposed-piston engine.

#### DETAILED DESCRIPTION OF VARIOUS EMBODIMENTS

FIG. 1 depicts an example of an opposed piston engine 10 including an arrangement of cylinders, pistons, and crankshafts with an associated gear train. The figure shows a three-cylinder arrangement, although this is not intended to be limiting; in fact, the basic architecture portrayed in FIG. 1 is applicable to opposed-piston engines with fewer, or more, cylinders. The opposed-piston engine 10 includes multiple cylinders 12, each cylinder 12 including exhaust ports 14 and intake ports 16. The cylinders may include liners (also called "sleeves") that are fixedly mounted in tunnels formed in an engine frame or block 18. A pair of pistons (not visible in this figure) is disposed for opposing reciprocal movement in a bore of each cylinder 12 (or in the cylinder liner). In the example of FIG. 1, the opposed-piston engine 10 includes an interlinked crankshaft system comprising two rotatably-mounted crankshafts 21 and 21a and a

crankshaft gear train 30 linking the crankshafts and coupling them to a power take-off shaft ("PTO shaft") 35. The crankshafts 21 and 21a are mounted to the engine, for example, by main bearing arrangements (not shown), one at the bottom of the engine block 18 and the other at the top. The crankshaft gear train 30 is supported in one end of the engine block 18 and is contained in a compartment 31 therein that can be accessed, for example, through a removable cover 32.

In FIG. 1, one piston of each piston pair is coupled to a respective crank journal 23 of the crankshaft 21 by a connecting rod assembly 27; the other piston is coupled to a respective crank journal 25 of the crankshaft 21a by a connecting rod assembly 29. The crankshafts 21 and 21a are disposed with their longitudinal axes in a spaced-apart, parallel arrangement. The crankshaft gear train 30 includes a plurality of gears, including, for example, two input gears 36a and 36b, which are fixed to respective ends of the crankshafts 21 and 21a for rotation therewith. In the embodiment illustrated in FIG. 1, an output gear 37 is mounted on the PTO shaft 3 and drives the PTO shaft 35 about an output axis of rotation A. In this configuration, two idler gears 39a and 39b are provided, each mounted for rotation on a fixed shaft or post 40. The idler gear 39a meshes with the input gear 36a and the output gear 37; the idler gear 39b meshes with the input gear 36b and the output gear 37. As a result of the configuration of the crankshaft gear train 30, the crankshafts 21 and 21a are co-rotating, that is to say, they rotate in a same direction. However, this is not meant to limit the scope of the present disclosure. In fact, a gear train construction according to the present disclosure may have fewer, or more, gears, and may have counter-rotating crankshafts. Thus, although five gears are shown for the crankshaft gear train 30, the numbers and types of gears for any particular crankshaft gear train are dictated by engine design. For example, the crankshaft gear train 30 may comprise one idler gear for counter-rotation, or two idler gears (as shown) for co-rotation.

FIG. 2 depicts an example of a portion of an opposed-piston engine 20 constructed for two stroke-cycle operation. The opposed-piston engine 20 includes a cylinder 22 with exhaust ports 24 and intake ports 26 formed in a sidewall 22w of the cylinder 22 near respective ends of the cylinder 22. The opposed-piston engine 20 includes at least the one cylinder 22, and may include two, three, or more cylinders similar to or different from the cylinder 22. The cylinder 22 may include a cylinder liner or sleeve supported in a block, a frame, a spar, or other structure. The cylinder sidewall 22w defines a cylindrical bore having a bore surface 28. Openings of the exhaust ports 24 and intake ports 26 are formed near respective ends of the sidewall 22w and open through the bore surface 28. A pair of pistons 34 and 36 is disposed for opposed sliding movement on the bore surface 28. Each of the pistons 34 and 36 is coupled by a respective connecting rod 38 (e.g., a portion of the connecting rod assembly 27 or 29 in FIG. 1) to a respective one of two crankshafts (e.g., as shown in FIG. 1). Each of the pistons 34 and 36 is equipped with one or more rings 41 that are mounted in annular grooves in crowns of the pistons 34 and 36.

The pistons 34 and 36 are shown at respective positions slightly after scavenging has commenced. The piston 34 has moved away from its bottom dead center (BDC) position at one end of the bore, and the exhaust ports are partially covered by the piston 34 but are still nearly fully open. The piston 36 has moved away from its BDC position at another end of the bore, and the intake ports 26 are partially covered by the piston 36. The exhaust ports 24 allow for transport of

exhaust gas out of the cylinder 22, and the intake ports 26 allow for transport of charge air into the cylinder 22. As motion of the pistons 34 and 36 continues, the piston 34 will move from its BDC location toward its top dead center (TDC) position in the interior of the bore, closing the exhaust ports 24. The piston 36 will continue to move from BDC toward its TDC position in the interior of the bore, closing the intake ports 26 as the piston 36 moves toward TDC. After the intake ports 26 and the exhaust ports 24 are closed, and as the pistons 34 and 36 continue to move closer together, charge air is compressed between end surfaces of the pistons 34 and 36. Fuel injected (e.g., through the sidewall 22w of the cylinder via injectors 42) mixes with the pressurized charge air, ignites, and drives pistons 34 and 36 from TDC to BDC in an expansion stroke.

During operation of the engine 20, the intake ports 26 and the piston 36 are exposed predominantly to charge air, while the exhaust ports 24 and the piston 34 are exposed to exhaust gas for extended periods of time. The exhaust gas is at a high temperature relative to the charge air. Prolonged and repeated exposure to exhaust gas throughout operation of the engine 20 can result in temperatures reached by the exhaust ports 24 and exhaust piston 34 at an exhaust end of the cylinder 22 being significantly greater than temperatures reached by the intake ports 26 and the piston 36 at an intake end of the cylinder 22. In an engine 20 where both pistons 34 and 36 are similarly constructed, such as with a similar structure and from the same materials, the piston design may not be optimal for one or both of the pistons 34 and 36 (e.g., the intake piston 36 may be over-designed for the intake temperatures, the exhaust piston 34 may be under-designed for the exhaust temperatures, or both). Such a non-optimal design can be costly in terms of materials, or in terms of life span of the exhaust piston 34.

According to embodiments of the present disclosure, exhaust pistons (e.g., the exhaust piston 34) are constructed differently from intake pistons (e.g., the intake piston 36). The exhaust pistons described below have features that allow an engine (e.g., the engine 10 or 20) to be compensated for, or adapted to, the different thermal conditions experienced at the intake end of the cylinder versus the exhaust end of the cylinder in a uniflow-scavenged opposed-piston engine, without sacrificing strength or cost.

FIG. 3A depicts an example of a piston 300 for use with a uniflow-scavenged opposed-piston engine. FIGS. 3B and 3C depict cross-sectional representations of the piston 300 shown in FIG. 3A. Specifically, FIG. 3B depicts a cross-sectional representation of the piston 300 through a plane that includes a longitudinal axis 312 of the piston 300 and a first cross-sectional axis 311, and FIG. 3C depicts a cross-sectional representation of the piston 300 through a plane that includes the longitudinal axis 312 of the piston 300 and a second cross-sectional axis orthogonal to the first cross-sectional axis 311. In one or more embodiments, the piston 300 can be used to implement pistons 34 and/or 36 in the opposed piston engine 20 discussed above in relation to FIG. 2.

Referring to FIG. 3A-3C, the piston 300 includes a crown 314 and a skirt part 316. In one or more embodiments, the crown 314 can be attached to, affixed to, or manufactured with the skirt part 316. For example, in one or more embodiments, the crown 314 can be welded to the skirt part 316. In some other embodiments, the crown 314 can be manufactured in a mold that is also used for manufacturing the skirt part 316.

The piston 300 includes a sidewall 318 which is generally cylindrical and extends along the longitudinal axis 312 from

an end 343 of the piston 300 to a first end 321 of the skirt part 316, and from the first end 321 to a second end 322 of the skirt part 316. The second end 322 of the skirt part 316 is structured to allow for engagement of a connecting rod 5 with the piston 300. The skirt part 316 defines a wristpin bore 324 in which a wristpin (not shown) is received and retained to engage the connecting rod with the wristpin. An outer peripheral surface of the crown 314 is formed with a first set of ring grooves 364. A second set of ring grooves 366 is formed in a portion of the sidewall 318 near the second end 322 of the skirt part 316. During engine operation, rings positioned in the piston ring grooves 364 and 366 prevent blow-by and undesirable burning of lubrication oil.

The sidewall 318 is formed with opposing sidewall portions 368 separated from one another by intervening sidewall indentations 370. For example, there are two opposing side wall sections 368 and two opposing indentations 370. Relative to the longitudinal axis 312, the portions 368 of the sidewall 318 have approximately a same radius as the crown 314. The indentations 370 can minimize both a mass of the piston and a contact area of the sidewall 318 against a bore of a cylinder in which the piston is disposed. The indentations 370 run longitudinally in the sidewall 318 between the first ring grooves 364 and the second ring grooves 366.

The crown 314 has an end surface 320 shaped to define a combustion chamber with an end surface of an opposing piston in the opposed-piston engine. In one or more embodiments, the end surface 320 can be a concave surface, a convex surface, a flat surface, or a combination thereof. The end surface 320 includes a depression 335 extending across the crown 314. Each end of the depression 335 is configured to align with a location of a respective fuel injector along the cylinder bore in which the piston 300 is disposed at a particular position of the piston 300 within the cylinder bore.

In one or more embodiments, the end surface 320 of the crown 314 can be formed of one or more materials such as titanium or titanium alloy. In one or more embodiments, the entire crown 314 can be formed of material such as titanium or titanium alloy. Titanium and titanium alloy have high R-value, and if used in the end surface 320 and/or the crown 314 can aid in confining the heat generated during combustion to the combustion chamber, and shield other parts of the engine. This in turn allows more of the heat generated in the combustion chamber to go into movement of the pistons and into maintaining suitable temperature of the exhaust gas.

In one or more embodiments, the end surface 320 of the crown 314 also includes a thermal barrier coating (TBC) 333, discussed further below in relation to FIG. 4. The TBC 333 confines heat generated during combustion to the combustion chamber, thus shielding other parts of the engine and allowing for more of the heat of combustion to go into movement of the pistons (and, when applicable, into heating the exhaust gas to a suitable temperature for treatment before recirculation). In one or more embodiments, the piston 300 may include only the titanium or titanium alloy end surface 320 (and/or a titanium/titanium alloy crown 314) without the TBC 333.

As shown in FIGS. 3B and 3C, the skirt part 316 includes an interior wall 323 that partially defines a cooling gallery 332. An outer peripheral portion of an under surface 336 of the crown 314 defines the remainder of the cooling gallery 332 in conjunction with the interior wall 323. The cooling gallery 332 serves as a conduit for cooling fluids such as oil to cool the piston 300.

As discussed above, intake and exhaust pistons in a pair of opposed pistons may differ in terms of structure, materials, or both. To account for the higher temperatures expe-

rienced by the exhaust piston, at least a portion of the exhaust piston may be made of one or more materials that are more suited to maintaining strength at higher temperatures than conventionally used materials such as steel or aluminum alloy. For example, in one or more embodiments, at least a portion of the exhaust piston may include titanium, a titanium alloy, a nickel alloy, a ceramic, a composite material, a cermet, or a combination of two or more of these. The exhaust piston may further include a thermal barrier coating, which in some embodiments is a layered or multi-component thermal barrier coating.

In one or more embodiments, in addition to including at least one material that is different from the materials used to form the intake piston, the exhaust piston may be shaped differently from the intake piston. For example, in one or more embodiments, the exhaust piston may have more or fewer structures than the intake piston to account for differences in coefficients of thermal expansion (CTE) between the intake piston and the exhaust piston. For example, in one or more embodiments, adequate clearance between the piston 300 and the cylinder bore in which the piston 300 is positioned can be provided by having a diameter of the sidewall 318 in the exhaust piston to be less than the diameter of the corresponding sidewall 318 in the intake piston. For another example, in one or more embodiments, shapes and sizes of the cooling galleries 332 can be different in the exhaust piston and the intake piston.

When two or more materials are used to construct the piston 300, differences in CTE associated with the different materials can impact a structural reliability of the piston 300. For example, CTE differences can cause deterioration or damage of the piston 300 at interfaces between materials, which in turn may lead to scuffing or seizing (or other types of wear) of the piston 300 in the cylinder bore within which the piston is disposed, in one or more embodiments, the exhaust piston can include coatings or materials between adjacent components (such as the skirt part 316 and the crown 314) formed of different materials, while such materials and coatings may be absent in the intake piston.

Differences in CTE additionally or alternatively may be present between the piston and its surroundings, such as between the piston rings and the engine cylinder liner (cylinder sleeve).

In one or more embodiments, the exhaust piston can include a piston skirt construction that is different from that of a corresponding piston skirt of the intake piston. The piston skirt construction for an exhaust piston can include a piston skirt that is made of a material that has a smaller coefficient of friction than the coefficient of friction of the material used to form the skirt of the intake piston. In one or more embodiments, materials that reduce friction between the cylinder bore and the piston skirt can include graphite and/or titanium with an interfacial layer of anodized or thermally grown titanium oxide. In some embodiments where the piston skirt includes titanium with anodized or thermally grown titanium oxide (e.g., titania), the titanium oxide can serve as a low friction material and can be provided on select portions of the piston skirt that can be expected to make contact with the cylinder. As shown in FIG. 3C, a low friction layer 337 is disposed on the sidewall 318, such as on the sidewall portions 368 of the skirt part 316 among other locations, where the low friction layer 337 can include the low friction materials discussed above.

In one or more embodiments, forming the exhaust piston and the intake piston with different materials may result in the pistons having different weights. For example, forming the exhaust piston with titanium or titanium alloys can result

in the exhaust piston weighing less than the intake piston, which may be formed using iron or stainless steel. In some instances, to maintain overall balance in the opposed-piston engine, it is desirable that the exhaust piston and the intake piston weigh about the same. To achieve substantially equal weights, in one or more embodiments, size or dimensions of the exhaust piston can be designed to achieve a weight of the exhaust piston that is substantially equal to a weight of the intake piston. For example, in embodiments where the 10 exhaust piston crown is manufactured using titanium or titanium alloys, the weight of the skirt part 316 can be increased such that the combined weight of the crown 314 and the skirt part 316 of the exhaust piston is substantially equal to the weight of crown 314 and the skirt part 316 of the intake piston. In one or more embodiments, the weight of the skirt part 316 can be increased by increasing a thickness of the skirt part 316 material.

As discussed above, in one or more embodiments, the exhaust piston can include a TBC 333 over the end surface 320 of the crown 314. In one or more embodiments, the TBC 333 can be partially made of a material with a high R-Value (R-Value is a measure of a material's resistance to heat flow). A TBC that includes a high R-Value material can aid in confining heat generated during combustion to the combustion chamber. This allows shielding other parts of the engine from the heat generated in the combustion chamber. Further, confining the heat to within the combustion chamber allows for more of the heat of combustion to be transformed into movement of the pistons and into heating the exhaust gas to a suitable temperature for treatment before recirculation (if applicable).

In one or more embodiments, the TBC 333 can include two or more layers of materials. In some such embodiments, alternating layers of the two or more materials can be used. 35 Any suitable technique or combination of techniques can be used to form the TBC 333. For example, in one or more embodiments, the TBC 333 can be formed using one or more of a casting technique, a thermal spraying technique, a physical deposition technique, additive manufacturing, and the like.

In one or more embodiments, the piston 300 also can include a bonding layer (e.g., bond-coat) between the end surface 320 of the piston 300 and the TBC 333. In one or more embodiments, the TBC 333 can include multiple bonding layers (e.g., bonding layers of varying grain or particulate size). In one or more embodiments, the portion of the TBC 333 that is deposited over the bonding layer, can include one or more layers of graduated material composition and one or more layers of homogenous material composition. A TBC 333 layer with graduated material composition can have material proportions that vary as a function of thickness of the TBC 333 layer; while a TBC 333 layer having homogeneous material composition can have material proportions that remain substantially constant over an entire thickness of the TBC 333 layer. When a bonding layer is used, the bonding layer can be of a metallic material or other material that adheres well to the bulk material of the piston 300 or piston crown 314, as well as to the material of the TBC 333. The material of the TBC 333 can be any suitable material with an R-Value, a softening temperature, or an operating temperature range that is acceptable for the environment in which the exhaust piston will be situated.

The TBC 333 can be a graduated coating; the coating can be a mixture of two or more materials, one of which can be a bonding material (e.g., the material used in the bonding layer or bond-coat). In a graduated thermal barrier coating, the concentration or amount of a first material (e.g., bonding

material) can be higher than that of a second material (e.g., material with a high R-Value) at the interface between the piston crown **314** and the thermal barrier coating. In such implementations, as one looks at the composition of the thermal barrier coating as a function of distance from the piston crown **314**, the concentration or amount of the first material will become less, or smaller, while the concentration or amount of the second material increases.

In one or more embodiments, an overall thickness of the TBC **333** may be approximately 1 mm in thickness. In some such implementations, the bonding layer can account for about 10% of the overall thickness of the TBC **333**. Alternatively, the bonding layer can have a thickness ranging from a few nanometers to about 100 microns. In some other embodiments, the bonding layer can be absent altogether. In 10 embodiments where the TBC **333** includes multiple sublayers of thermal barrier material of differing composition or structure, the overall thickness of the sublayers can be about 90% or more of the overall thickness of the TBC **333**. In 15 such an assemblage, each individual layer can have the same thickness or each layer can have a different thickness. In one or more embodiments, one sublayer can differ from another sublayer in terms of one or more of crystal structure of the material, material density or porosity, and grain or particle size.

FIG. 4 depicts a cross-sectional representation of a thermal barrier coating **400** disposed over an example piston for use with a uniflow-scavenged opposed-piston engine. In one or more embodiments, the TBC **400** can be used to implement the TBC **333** discussed above in relation to FIGS. 3A-3C. The TBC **400** includes a bonding layer **402** and a thermal barrier layer **404**. The bonding layer **402** is disposed on an end **401** of a piston while the thermal barrier layer **404** is disposed over the bonding layer **402**. The bonding layer **402** includes a first bonding sublayer **402a** and a second bonding sublayer **402b**. The thermal barrier layer **404** includes a first **404a**, a second **404b**, a third **404c**, and a fourth **404d** thermal barrier sublayer. In one or more embodiments, the TBC **400** may not include a bonding layer **402**, and instead have the thermal barrier layer **404** directly disposed on the end **401** of the piston.

In one more embodiments, the bonding layer **402** can include materials that have CTE close to the CTE of the material used to form the piston and the CTE of the material used to form the thermal barrier layer **404**. For example, in one or more embodiments, the CTE of a bonding material used for forming the bonding layer **402** is within about 5% to about 10% of the CTE of the material used for forming the piston, and is within 5% to about 10% of the CTE of a material used for forming the thermal barrier layer **404**. In one or more embodiments, the bonding material used for forming the bonding layer **402** can include a metal. In one or more embodiments, a coarseness of the bonding material used on the first bonding sublayer **402a** can be different from a coarseness of the bonding material used in the second bonding sublayer **402b**. For example, the bonding material used in the second bonding sublayer **402b** can be coarser than that used in the first bonding sublayer **402a**. In one or more embodiments, a thickness of the first bonding sublayer **402a** can be different from a thickness of the second bonding sublayer **402a**. In one or more embodiments, the first bonding sublayer **402a** can be thicker than the second bonding sublayer **402b**. For example, in one or more embodiments, the thickness of the first bonding sublayer **402a** can be about 50 microns to about 100 microns, or about 75 microns, and the thickness of the second bonding sublayer **402b** can be about 10 microns to about 35 microns, or

about 25 microns. In one or more embodiments, the bonding material can include an oxidation-resistant metal or metal alloy, such as, for example, nickel-chromium-aluminum-yttrium (NiCrAlY) and/or nickel-cobalt-chromium-aluminum-yttrium (NiCoCrAlY).

In one or more embodiment, the thermal barrier layer **404** can include ceramic materials. For example, in some such embodiments, the thermal barrier layer **404** can include yttria stabilized zirconia (YSZ). YSZ has a high R-value, is 10 stable over a wide range of temperatures, and has mechanical properties that are well suited for use in an internal combustion engine. In one or more embodiments, the thermal barrier layer **404** can include a bonding material in 15 addition to the ceramic material. The inclusion of bonding material can improve the adhesion of the thermal barrier layer **404** to the underlying layers and can help in matching the overall CTE of the thermal barrier layer **404** with the CTE of the end **401** of the piston. For example, in one or 20 more embodiments, the thermal barrier layer **404** can have graduated relative concentrations of the bonding material and the ceramic material over the thickness of the thermal barrier layer **404**. In one such example, the concentration of the bonding material can decrease while the concentration of the ceramic material can increase from the first thermal 25 barrier sublayer **404a** through the fourth thermal barrier sublayer **404d**. Specifically, for example, the first thermal barrier sublayer **404a** can have a composition, by weight, of about 75% bonding material and about 25% ceramic material; the second thermal barrier sublayer **404b** can have a 30 composition, by weight, of about 50% bonding material and about 50% ceramic material; the third thermal barrier sublayer **404c** can have a composition, by weight, of about 25% bonding material and about 75% ceramic material; and the fourth thermal barrier sublayer **404d** can have a composition, by weight, of about 5% bonding material and about 95% ceramic material. Alternatively, in one or more embodiments, the fourth barrier sublayer **404d** can have a composition, by weight, of about 0% bonding material and about 100% ceramic material. The above mentioned relative concentrations of the bonding material and the ceramic material are only examples, and other relative concentrations can be used as appropriate, in some other embodiments, one or more materials such as mullite, alumina, and rare-earth zirconates can be used in place of or in addition to YSZ.

In one or more embodiments, the thickness of one or more sublayers of the thermal barrier layer **404** can be different from the thickness of another sublayer of the thermal barrier layer **404**. For example, in some such embodiments, the thickness of the first thermal barrier sublayer **404a** can be about 50 microns to about 150 microns, or about 100 microns. The thickness of the second thermal barrier sublayer **404b** can be about 25 microns to about 75 microns, or about 50 microns. The thickness of the third thermal barrier sublayer **404c** can be about 25 microns to about 75 microns, or about 50 microns. The thickness of the fourth thermal barrier sublayer **404d** can be about 500 microns to about 900 microns, or about 700 microns. In one or more embodiments, the thickness of the fourth thermal barrier sublayer **404d** can be greater than the thickness of each of the other 50 sublayers of the thermal barrier layer **404**.

FIG. 5 shows a flow chart of an example method **500** for forming a thermal barrier coating on a piston. In one or more embodiments, the process **500** can be used to form the TBC **333** or the TBC **400** discussed above in relation to FIGS. 3A-3C and FIG. 4, respectively. The process **500** includes providing a piston of an opposed-piston engine (at **502**). In one or more embodiments, providing a piston can include

## 11

providing an exhaust piston of an opposed piston engine similar to the piston 300 discussed above in relation to FIGS. 3A-3C. The piston can include a skirt and a crown having an end surface, similar to the skirt part 316, the crown 314 and the end surface 320 of the piston 300. In one or more embodiments, the end surface 320 and/or the crown 314 can be made of materials such as titanium and/or titanium alloy. The method 500 further includes preparing the end surface of the piston for deposition of a thermal barrier coating (at 504). In one or more embodiments, preparing the end surface can include cleaning, polishing, roughening, etching, annealing, or any combination thereof. Such preparation can improve adhesion of the thermal barrier layer onto the prepared end surface of the piston.

The process 500 also includes disposing a bonding material over the prepared end surface (at 506). As discussed above in relation to FIG. 4, the bonding layer 402 can include bonding materials such as metal or metal alloys. Further the bonding layer 402 can include two or more sublayers, where each sublayer can have different properties such as thickness and/or coarseness of the bonding material. In one or more embodiments, the bonding material can be deposited on the end surface of the piston using one or more of a casting technique, a thermal spraying technique, a physical deposition technique, additive manufacturing techniques, and electrochemical deposition technique.

The process 500 further includes depositing a thermal barrier material over the bonding material (at 508). The thermal barrier material can include materials such as ceramics and other high R-value materials. In one or more embodiments, the thermal barrier layer can be deposited over the bonding material to form a thermal barrier layer similar to the thermal barrier layer 404 discussed above in relation to FIG. 4. In particular, the thermal barrier layer can include multiple sublayers composed of varying proportions of a bonding material and a thermal barrier material such as ceramic. In one or more embodiments, the thermal barrier material can be deposited on the bonding material using one or more of a casting technique, a thermal spraying technique, a physical deposition technique, additive manufacturing techniques, and an electrochemical deposition technique.

The process 500 may also include treating the piston after the deposition of the thermal barrier material. For example, in one or more embodiments, the piston can undergo an annealing process to improve the adhesion between the thermal barrier material and the bonding material. The annealing process can also improve the mechanical properties of the TBC by relieving post deposition shear stress within the deposited layers of thermal barrier material. In one or more embodiments, the piston can undergo further post TBC deposition processing such as oxidation of selected surfaces of the piston. For example, sidewall surfaces of the skirt part 316 (FIG. 3B) can be oxidized to create a low friction surface.

FIG. 6 shows a flow chart of an example method 600 for forming a thermal barrier coating on a piston (e.g., the piston 300 or the piston 700 described with respect to FIG. 7) according to another embodiment. In one or more embodiments, the process 600 can be used to form the TBC 333 or the TBC 400 discussed above in relation to FIGS. 3A-3C and FIG. 4, respectively. The process 600 includes providing a piston of an opposed-piston engine (at 602). In one or more embodiments, providing a piston can include providing an exhaust piston of an opposed piston engine similar to the piston 300 discussed above in relation to FIGS. 3A-3C. The piston can include a skirt and a crown having an end surface,

## 12

similar to the skirt part 316, the crown 314, 714 and the end surface 320, 720 of the piston 300, 700. In one or more embodiments, the end surface 320, 720 and/or the crown 314, 714 can be made of materials such as titanium and/or titanium alloy. In some embodiments, the method 600 also includes preparing the end surface of the piston for deposition of a thermal barrier coating (at 604). In one or more embodiments, preparing the end surface can include cleaning, polishing, roughening, etching, annealing, or any combination thereof. Such preparation can improve adhesion of the thermal barrier layer onto the prepared end surface of the piston.

The process 600 also includes depositing a bonding layer including a bonding material on the end surface (e.g., the prepared end surface) using a high velocity oxy-fuel (HVOF) spray process, (at 606). As discussed above in relation to FIG. 4, the bonding layer 402 can include bonding materials such as metal or metal alloys. Furthermore, the bonding layer 402 can include two or more sublayers, where each sublayer can have different properties such as thickness and/or coarseness of the bonding material. The HVOF spray process comprises spraying a molten or semi-molten spray of the bonding material (e.g., NiCo-CrAlY or any other bonding material described herein) on the end surface using a high temperature and high velocity gas stream so as to produce a dense coating of the bonding layer. In particular embodiments, the HVOF spray may comprise a stream of the bonding material having a predetermined diameter. A plurality of line passes of the HVOF spray may be performed on the end surface (e.g., the end surface 320, 720) so as to sequentially coat the entire end surface with the bonding layer. In other embodiments, multiple line passes of the HVOF spray may be performed over previously deposited bonding layers, for example, to obtain a desired thickness of the bonding layer on the end surface (e.g., the end surface 320, 720).

The process 600 further includes depositing at least one thermal barrier layer comprising ceramic material over the bonding material, (at 608). In particular embodiments, the thermal barrier layer is deposited using an atmospheric plasma spray process. For example, the piston (e.g., the piston 300, 700) may be positioned in a vacuum chamber. One or more processing gases may be introduced into the vacuum chamber in the presence of an electric arc which ionizes the processing gases so as to form a plasma. Powdered feedstock of a thermal barrier material (e.g., YSZ or any other ceramic material described herein) may be introduced into the vacuum chamber along with the plasma. The thermal barrier material may be melted by the plasma and propelled towards the piston, for example, the end surface 320, 720 of the pistons 300, 700 so as to deposit thereon and form the thermal barrier layer. In particular embodiments, multiple rounds of the atmospheric plasma spray process may be performed, for example, to obtain a desired thickness of the thermal barrier layer on the end surface.

The thermal barrier material can include materials such as ceramics and other high R-value materials. In one or more embodiments, the thermal barrier layer can be deposited over the bonding material to form a thermal barrier layer similar to the thermal barrier layer 404 discussed above in relation to FIG. 4. In particular, the thermal barrier layer can include multiple sublayers composed of varying proportions of a bonding material and a thermal barrier material such as ceramic. In various embodiments, the ceramic material comprises YSZ in the range of 7 wt % to 9 wt % (e.g., 7 wt %, 8 wt % or 9 wt % inclusive of all ranges and values therebetween).

The process 600 may also include treating the piston after the deposition of the thermal barrier material. For example, in one or more embodiments, the piston can undergo an annealing process to improve the adhesion between the thermal barrier material and the bonding material. The annealing process can also improve the mechanical properties of the TBC by relieving post deposition shear stress within the deposited layers of thermal barrier material. In one or more embodiments, the piston can undergo further post TBC deposition processing such as oxidation of selected surfaces of the piston. For example, sidewall surfaces of the skirt part 316 (FIG. 3B) can be oxidized to create a low friction surface. In other embodiments, post-processing may include polishing the bonding layer before deposition of the thermal barrier layer and/or polishing the thermal barrier layer so as to increase uniformity or homogenize a thickness of the bonding layer and/or the thermal barrier layer.

FIG. 7 is a perspective view of a piston 700 for use with a uniflow-scavenged opposed-piston engine, according to a particular embodiment. In one or more embodiments, the piston 700 can be used to implement pistons 34 and/or 36 in the opposed piston engine 20 discussed above in relation to FIG. 2. The piston 700 includes a crown 714 and may also include a skirt part (not shown), for example the skirt part 316. In one or more embodiments, the crown 714 can be attached to, affixed to, or manufactured with the skirt part. For example, in one or more embodiments, the crown 714 can be welded to the skirt part (e.g., the skirt part 316). In other embodiments, the crown 614 can be manufactured in a mold that is also used for manufacturing the skirt part (e.g., the skirt part 316).

The crown 714 has an end surface 720 shaped to define a combustion chamber with an end surface of an opposing piston in the opposed-piston engine. The end surface 720 comprises a rim portion 721 which forms a perimeter of the end surface 720. The rim portion may be substantially flat. A plurality of depressions 735 may extend across the rim portion 721. Each end of the depressions 735 may be configured to align with a location of a respective fuel injector along the cylinder bore in which the piston 700 is disposed at a particular position of the piston 700 within the cylinder bore.

In one or more embodiments, the end surface also defines a trough 722 formed radially inwards of the rim portion 721. While shown as having a concave surface, in other embodiment, the trough may have a convex surface, a flat surface, or a combination thereof. The end surface 720 also comprises a dome portion 715 positioned axially around a central axis of the piston 700.

The end surface 720 of the crown 714 can be formed of one or more materials such as titanium or titanium alloy. In one or more embodiments, the entire crown 714 can be formed of a material such as titanium or titanium alloy. Titanium and titanium alloy have high R-value, and if used in the end surface 720 and/or the crown 714 can aid in confining the heat generated during combustion to the combustion chamber and shield other parts of the engine. This in turn allows more of the heat generated in the combustion chamber to go into movement of the pistons and into maintaining suitable temperature of the exhaust gas.

The end surface 720 of the crown 714 may also include a TBC (e.g., the TBC 333 or a combination of the bonding layer 402 and the thermal barrier layer 404), as previously described herein. The TBC confines heat generated during combustion to the combustion chamber, thus shielding other parts of the engine and allowing for more of the heat of

combustion to go into movement of the pistons (and, when applicable, into heating the exhaust gas to a suitable temperature for treatment before recirculation). In one or more embodiments, the piston 700 may include only the titanium or titanium alloy end surface 720 (and/or a titanium/titanium alloy crown 714) without the TBC.

FIG. 8 is an image of a coating assembly 80 for depositing a bonding layer (e.g., the bonding layer 402) and/or a thermal barrier layer (e.g., the thermal barrier layer 404) on the piston 700 or any other piston (e.g., the piston 300) described herein. The coating assembly 80 includes a chuck 82 for mounting the piston 700 or any other piston (e.g., the piston 300 thereon). While only the crown 714 of the piston 700 is shown mounted on the chuck 82, in other embodiments, the chuck 82 may be structured to mount the piston 700 with a skirt coupled to the crown 714.

A plasma torch 84 is mounted on a six-axis robot 86 and configured to produce a HVOF spray of the bond coat material over the end surface 720 of the crown 714. The plasma torch may be translated linearly over the end surface 720 so as to perform a plurality of line passes of the HVOF spray of the bonding material and/or the thermal barrier material on the end surface 720 so as to deposit a bonding layer (e.g., the bonding layer 402) and/or thermal barrier layer (e.g., the thermal barrier layer 404). Furthermore, the chuck 82 may be rotatable (e.g., mounted on a rotation table). In various embodiments, rotation of the chuck 82 causes the piston to rotate during or in-between the line passes of the HVOF spray. This may allow re-orientation of the end surface 720 relative to the plasma torch 84, for example, to allow more uniform coating of the end surface with the bonding layer (e.g., the bonding layer 402) and/or the thermal barrier layer (e.g., the thermal barrier layer 404). Multiple line passes of the HVOF spray of the bonding material and/or the thermal barrier layer may be performed on the same area of the end surface 720 so as to obtain a desired thickness of the bonding layer on various portions of the bond surface. In other embodiments, the thermal barrier layer (e.g., the thermal barrier layer 404) may then be coated on the bonding layer, for example using the atmospheric plasma spray process.

As shown in FIG. 7, the end surface 720 of the piston 700 includes curvatures and out of plane regions. Particularly, the trough 722 is formed as a cavity in the end surface 720, and it may be difficult to get a uniform coating and/or a coating of a desired thickness on the various portions of the end surface 720, for example, the curved surfaces and/or corners of the trough 722. In various embodiments, a portion of the end surface 720 may be masked (e.g., covered with a barrier) during an initial bonding layer and/or thermal barrier layer deposition process. For example, FIG. 9 shows a mask 90 positioned in the trough 722 of the end surface 720. The mask 90 prevents the bonding material and/or the thermal barrier layer from being deposited in the trough 722 (e.g., a base of the trough 722) or portions thereof, while the open portions of the end surface 720 are coated with the bonding layer and/or thermal barrier layer.

Once a desired thickness of the bonding layer and/or the thermal barrier layer is achieved on the open portions, the mask 90 may be removed, and the bonding layer and/or thermal barrier layer may be coated on the unmasked portion, for example, the base of the trough 722. In particular embodiments, the bonding material may be deposited for a first predetermined time on the unmasked portion (e.g., the trough 722) after the open portions have been coated, for example, to obtain a desired thickness of the bonding layer thereon. Similarly, the thermal barrier material may be

deposited for a second predetermined time on the unmasked portion (e.g., the trough 722) after the open portions have been coated, for example, to obtain a desired thickness of the thermal barrier layer thereon.

FIG. 10 shows a flow chart of an example method 1000 for forming a thermal barrier coating on a piston (e.g., the piston 300, 700), according to another embodiment. In one or more embodiments, the method 1000 can be used to form the TBC 333 or the TBC 400 discussed above in relation to FIGS. 3A-3C and FIG. 4, respectively. The method 1000 includes providing a piston of an opposed-piston engine (at 1002). In one or more embodiments, providing a piston can include providing an exhaust piston of an opposed piston engine similar to the piston 300 or 700 as discussed above in relation to FIGS. 3A-3C and FIG. 7, respectively. The piston can include a skirt and a crown having an end surface, similar to the skirt part 316, the crown 314, 714 and the end surface 320, 720 of the piston 300, 700. In one or more embodiments, the end surface 320, 720 and/or the crown 314, 714 can be made of materials such as titanium and/or titanium alloy. In some embodiments, the method 1000 may further include preparing the end surface of the piston for deposition of a thermal barrier coating (at 1004). In one or more embodiments, preparing the end surface can include cleaning, polishing, roughening, etching, annealing, or any combination thereof. Such preparation can improve adhesion of the thermal barrier layer onto the prepared end surface of the piston.

The method 1000 includes masking a portion of the end surface, (at 1006). For example, as discussed with respect to FIGS. 8-9, the trough 722 or any other portion of the end surface 720 of the piston 700 may be covered with the mask 90. The mask may include a physical barrier (e.g., a metal piece or strip, a tube positioned in the trough 722, etc.) or a sacrificial coating (e.g., a coating of a chemical such as a photoresist which may be removed by dissolving in a solvent).

The method 1000 also includes depositing a bonding layer including a bonding material over the end surface (e.g., the prepared end surface) (at 1008). The bonding material may be deposited using the FI OF spray process, and may include the bonding layer 402 or any other bonding layer described herein. In particular embodiments, the bonding material may be deposited using a spray nozzle having a nozzle diameter in a range of 5 mm to 8 mm. The mask prevents the bonding material from being deposited on the masked portions of the end surface, such that the bonding layer is deposited only on the open areas of the end surface (e.g., the rim portion 721 and the dome portion 715) of the end surface (e.g., the end surface 720). A plurality of line passes of the HVOF spray may be performed on the end surface (e.g., the end surface 320, 720) so as to sequentially coat the entire end surface with the bonding layer. In other embodiments, multiple line passes of the HVOF spray may be performed over a previously deposited bonding layer, for example, to obtain a desired thickness of the bonding layer on the end surface (e.g., the end surface 320, 720).

The portion of the end surface is unmasked (at 1010). For example, the mask 90 is removed from the trough 722 after the initial bonding layer is deposited. The bonding material is deposited over at least the portion of the end surface for a first predetermined time (at 1012). For example, the mask 90 may be removed and the bonding material may be deposited at least in the trough 722 for the first predetermined time (e.g., in a range of 5 seconds to 20 seconds).

In some embodiments, the method 1000 also includes masking the portion of the end surface before depositing at

least one thermal barrier material comprising ceramic material above the bonding material (at 1014). For example, once the bonding layer has been deposited on the end surface, the mask (e.g., the mask 90) may again be disposed on the portion of the end surface (e.g., the trough 722 of the end surface 720). At least one thermal barrier material comprising ceramic material is deposited above the bonding layer (at 1016). For example, the thermal barrier layer 404 is deposited on the open portions (e.g., the rim portion 721 and the dome portion 715) of the end surface (e.g., the end surface 720).

In some embodiments, the thermal barrier material is deposited using an atmospheric plasma spray process. In other embodiments, the thermal barrier material may be deposited over the bonding layer using the HVOF spray process (e.g., via a plurality of lines passes of the HVOF spray of the thermal barrier material). In particular embodiments, multiple rounds of the atmospheric plasma spray process or the HVOF spray may be performed, for example, to obtain a desired thickness of the thermal barrier layer on the end surface. The thermal barrier material can include materials such as ceramics and other high R-value materials. In one or more embodiments, the thermal barrier layer can be deposited over the bonding material to form a thermal barrier layer similar to the thermal barrier layer 404 discussed above in relation to FIG. 4. In particular, the thermal barrier layer can include multiple sublayers composed of varying proportions of a bonding material and a thermal barrier material such as ceramic. In various embodiments, the ceramic material comprises YSZ in the range of 7 wt % to 9 wt % (e.g., 7 wt %, 8 wt % or 9 wt % inclusive of all ranges and values therebetween).

The portion of the end surface is unmasked (at 1018). For example, the mask 90 is removed from the trough 722. The at least one thermal barrier comprising ceramic material is deposited over the bonding layer coated on the portion of the end surface for a second predetermined time (at 1020). For example, the mask 90 may be removed and the thermal barrier layer may be deposited at least in the trough 722 for the second predetermined time (e.g., in a range of 5 seconds to 20 seconds).

In various embodiments, the method 1000 may also include treating the piston after the deposition of the thermal barrier material. For example, in one or more embodiments, the piston 700 can undergo an annealing process to improve the adhesion between the thermal barrier material and the bonding material. The annealing process can also improve the mechanical properties of the TBC by relieving post deposition shear stress within the deposited layers of thermal barrier material. In one or more embodiments, the piston can undergo further post TBC deposition processing such as oxidation of selected surfaces of the piston. For example, sidewall surfaces of the skirt part 316 (FIG. 3B) can be oxidized to create a low friction surface. In other embodiments, post-processing may include polishing the bonding layer before deposition of the thermal barrier layer and/or polishing the thermal barrier layer so as to increase uniformity or homogenize a thickness of the bonding layer and/or the thermal barrier layer.

As discussed above, a piston for use in a uniflow-scavenged opposed-piston engine that includes at least one cylinder includes features for adapting the engine to variations in thermal conditions between an intake end and an exhaust end of the cylinder in the opposed-piston engine.

For the purpose of this disclosure, the term "coupled" means the joining of two members directly or indirectly to one another. Such joining may be stationary or moveable in

nature. Such joining may be achieved with the two members or the two members and any additional intermediate members being integrally formed as a single unitary body with one another or with the two members or the two members and any additional intermediate members being attached to one another. Such joining may be permanent in nature or may be removable or releasable in nature.

It should be noted that the orientation of various elements may differ according to other exemplary embodiments, and that such variations are intended to be encompassed by the present disclosure. It is recognized that features of the disclosed embodiments can be incorporated into other disclosed embodiments.

It is important to note that the constructions and arrangements of apparatuses or the components thereof as shown in the various exemplary embodiments are illustrative only. Although a few embodiments have been described in detail in this disclosure, those skilled in the art who review this disclosure will readily appreciate that many modifications are possible (e.g., variations in sizes, dimensions, structures, shapes and proportions of the various elements, values of parameters, mounting arrangements, use of materials, colors, orientations, etc.) without materially departing from the novel teachings and advantages of the subject matter disclosed. For example, elements shown as integrally formed may be constructed of multiple parts or elements, the position of elements may be reversed or otherwise varied, and the nature or number of discrete elements or positions may be altered or varied. The order or sequence of any process or method steps may be varied or re-sequenced according to alternative embodiments. Other substitutions, modifications, changes and omissions may also be made in the design, operating conditions and arrangement of the various exemplary embodiments without departing from the scope of the present disclosure.

While various inventive embodiments have been described and illustrated herein, those of ordinary skill in the art will readily envision a variety of other mechanisms and/or structures for performing the function and/or obtaining the results and/or one or more of the advantages described herein, and each of such variations and/or modifications is deemed to be within the scope of the inventive embodiments described herein. More generally, those skilled in the art will readily appreciate that, unless otherwise noted, any parameters, dimensions, materials, and configurations described herein are meant to be exemplary and that the actual parameters, dimensions, materials, and/or configurations will depend upon the specific application or applications for which the inventive teachings is/are used. Those skilled in the art will recognize, or be able to ascertain using no more than routine experimentation, many equivalents to the specific inventive embodiments described herein. It is, therefore, to be understood that the foregoing embodiments are presented by way of example only and that, within the scope of the appended claims and equivalents thereto, inventive embodiments may be practiced otherwise than as specifically described and claimed. Inventive embodiments of the present disclosure are directed to each individual feature, system, article, material, kit, and/or method described herein. In addition, any combination of two or more such features, systems, articles, materials, kits, and/or methods, if such features, systems, articles, materials, kits, and/or methods are not mutually inconsistent, is included within the inventive scope of the present disclosure.

Also, the technology described herein may be embodied as a method, of which at least one example has been

provided. The acts performed as part of the method may be ordered in any suitable way unless otherwise specifically noted. Accordingly, embodiments may be constructed in which acts are performed in an order different than illustrated, which may include performing some acts simultaneously, even though shown as sequential acts in illustrative embodiments.

The claims should not be read as limited to the described order or elements unless stated to that effect. It should be understood that various changes in form and detail may be made by one of ordinary skill in the art without departing from the spirit and scope of the appended claims. All embodiments that come within the spirit and scope of the following claims and equivalents thereto are claimed.

The invention claimed is:

1. A method of making a piston for an opposed-piston engine, the method comprising:

providing a piston, the piston comprising a piston crown located at an end of the piston, the piston crown comprising:

a cylindrical portion including a sidewall; and an end surface structured to form a combustion chamber when disposed within a cylinder bore in cooperation with an end surface of a cooperating opposing piston;

masking a portion of the end surface;

depositing a bonding layer including a bonding material

on the end surface of the piston crown;

unmasking the portion of the end surface;

depositing the bonding layer on at least the portion of the end surface for a first predetermined time; and depositing at least one thermal barrier layer comprising ceramic material above the bonding layer.

2. The method of claim 1, wherein the at least one thermal barrier layer is deposited using an atmospheric plasma spray.

3. The method of claim 2, wherein depositing at least one thermal barrier layer comprises ceramic material above the bonding layer comprises depositing a plurality of thermal barrier sublayers, each of the plurality of thermal barrier sublayers including a proportion of the ceramic material and a proportion of the bonding material, wherein the proportion of the ceramic material decreases and the proportion of the bonding material increases with the depth of the thermal barrier layer.

4. The method of claim 3, wherein depositing a plurality of thermal barrier sublayers comprises depositing at least one sublayer of the plurality of thermal barrier sublayers with a thickness that is different from a thickness of another sublayer of the plurality of thermal barrier sublayers.

5. The method of claim 2, wherein depositing at least one thermal barrier layer comprises ceramic material above the bonding layer comprises depositing a ceramic material including at least one of yttria stabilized zirconia, mullite, alumina, and rare-earth zirconates.

6. The method of claim 5, wherein the ceramic material comprises yttria stabilized zirconia in a range of 7 wt % to 9 wt %.

7. The method of claim 2, wherein the at least one thermal barrier layer is deposited using a plurality of the atmospheric plasma spray.

8. The method of claim 2, wherein providing a piston comprises providing the piston where the end surface comprises at least one of steel, aluminum alloy, titanium, a titanium alloy, or a nickel alloy.

9. The method of claim 1, wherein the bonding material is deposited using a high velocity oxy-fuel spray.

**10.** The method of claim **9**, wherein depositing the bonding layer comprises providing a plurality of line passes of the high velocity oxy-fuel spray.

**11.** The method of claim **1**, further comprising:  
masking the portion of the end surface before depositing <sup>5</sup>  
the at least one thermal barrier material comprising  
ceramic material above the bonding material; and  
unmasking the portion of the end surface; and  
depositing the at least one thermal barrier comprising  
ceramic material over the bonding layer coated on the <sup>10</sup>  
portion of the end surface for a second predetermined  
time.

\* \* \* \* \*